

## UNITED STATES PATENT OFFICE

2,364,702

## ELECTRICAL CONDUCTOR

Donald Finlayson, Ernest Leslie Greenwood, and William John Simpson, Spondon, near Derby, England, assignors to British Celanese Limited, London, England, a company of Great Britain

No Drawing. Application August 4, 1942, Serial No. 453,558. In Great Britain July 7, 1941

3 Claims. (Cl. 57—162)

This invention relates to electrical conductors and is particularly concerned with the insulation of wires for this purpose.

The invention is primarily concerned with the insulation of very fine wires, particularly of the order of 33 to 50 S. W. G. (British standard wire gauge) corresponding to wire diameters of 0.010" to 0.001" and approximately to 29 to 40 American wire gauge (B and S), although of course the present invention may be applied to wires of coarser gauge.

For the insulation of such wires, two standard methods are available; firstly the wire may be lapped or wound with a covering of silk filaments, and secondly the wire may be covered with a coating of varnish or enamel. The latter method is subject to the possibility of minute pin-holes which render it unreliable, presents difficulties in obtaining uniformity of coating owing to a tendency of the applied material to run in the liquid state to one side of the wire or along the length of the wire, and further cannot always be used in conditions where the wire is subjected for long periods to even moderately high temperatures. The method of lapping with a covering of silk filaments is expensive on account of the high price of silk, and, moreover, if the silk lapping is damaged locally the filaments may run back so that the insulation is impaired beyond the point at which damage occurs. Instead of silk filaments, the continuous artificial filaments, e. g. filaments of cellulose acetate, have been used for this purpose, and although they are less expensive than silk they are subject to the other disadvantages of silk mentioned above. In addition, the only materials of this kind available on a commercial scale have been of a denier of the order of 2.5 and upwards which gives them a lower covering power than the relatively finer silk filaments. Again, both with silk and with artificial silk filaments of the denier mentioned, the tension applied to the filaments in the course of the lapping operation is such that the filaments tend to cut into the very fine wires employed, or at least to impose upon them such a strain as causes the wire to be forced from a straight configuration into a slightly helical form.

It has been proposed to cover wires with artificial filaments of organic derivatives of cellulose such as cellulose acetate and to coalesce the filaments partially or completely in order to impart a continuous and relatively waterproof surface to the layer or layers of filaments after they have been lapped upon the wire. So far as we

are aware, however, this method has met with no commercial success, presumably on account of the fact mentioned above that the filaments commercially available were of too coarse a denier.

Further investigation and research into this problem have shown that fine wires can be efficiently insulated by lapping them with artificial filaments of a thermoplastic material having electrically insulating properties, provided that filaments of lower denier than those heretofore available are used and that the filaments are coalesced to form a continuous insulating cover for the wire.

While filaments of a denier of less than 1.5 and if desired very much less, e. g. of the order of 0.5 denier or less, may be produced by stretching coarser filaments of a thermoplastic material in the presence of a softening agent to twice, or 15 five, ten, or more times their original length, the filaments produced in this way have a very much reduced extensibility which gives rise to difficulties in the lapping operation. Moreover, while this low extensibility may be increased by 20 subjecting the stretched yarn to a shrinking operation, such a step involves increasing unduly the cost of the filaments, which is already high by reason of the cost of the stretching step itself. For these reasons it is preferred to spin 25 the filaments to the required low denier in the first instance, i. e. in the course of the operation of forming the filaments by extruding a spinning solution through fine orifices. This, it has been found, is made possible in the case of cellulose acetate filaments by the use of a spinning solution of low concentration and consequently of low viscosity.

The fine artificial filaments employed for the purpose of the present invention may be of any 30 filament-forming organic substance having a high electrical resistance and capable of being softened to bring about coalescence without impairing the insulating properties of the substance of the filaments. As previously mentioned, a 35 suitable material for use as the basis of the filaments is cellulose acetate. Other organic derivatives of cellulose may be employed such as other cellulose esters, e. g. cellulose propionate and butyrate, mixed esters such as cellulose acetate-propionate and acetate-butyrate, or cellulose ethers such as ethyl and benzyl cellulose.

In the lapping operation the filaments are 40 preferably employed in the form of a thread or bundle having at most very little twist and preferably no twist at all. The difficulty of collect-

ing a completely untwisted bundle of fine filaments in the course of spinning may be overcome by taking up the filaments as they are extruded on large-diameter take-up means, e. g. on metal swifts of, say, 45" circumference, the take-up package serving to control the spinning speed by drawing the filaments directly away from the point of extrusion, and subsequently serving as supply packages for the winding of the cheeses or other special packages to be used in the lapping operation. Thus, the filaments wound off the swift above mentioned may be wound into cheeses of, say, from  $\frac{1}{8}''$ - $2\frac{1}{2}''$  in length,  $\frac{1}{8}''$ - $\frac{1}{2}''$  internal diameter, and  $1\frac{1}{8}''$ - $2''$  external diameter, according to the requirements of the machine on which lapping is to take place. By these means it is possible to effect the spinning and re-winding of filaments having a denier of unity or less, in the form of bundles having a total denier of 22 or less, though for most purposes filament bundles of from 30 to 150 denier are required. The spinning and winding operation is facilitated by the application of a suitable lubricant to the bundle, an example of which is a solution containing 20% by weight of triethanolamine oleate, 5% oleic acid and 75% mineral oil.

By the use of a twistless bundle of fine filaments produced in the manner described above, wires can be lapped by the methods employed in the silk lapping of wires, though care is necessary if the operation is to be conducted at the same speed as is employed for silk lapping. For example, it is desirable to eliminate, in the guiding surfaces of the lapping machine, roughnesses that might be tolerable in connection with silk, and, further, it is generally better to use a lower tension in the filament bundle than is the practice with silk. The necessity of the last-mentioned precaution is not wholly disadvantageous, since it eliminates the defects sometimes experienced in silk lapping, due to the tension in the silk reacting after lapping, on the wire itself, forcing it out of the straight into a slightly helical shape. Apart from these points, however, the invention enables certain advantages to be obtained by departing from the methods ordinarily employed in silk lapping. The size of the bundle employed in the ordinary practice of silk lapping wires of from 18 to 48 gauge is of the order of 30-100 denier. The denier is roughly proportional to the diameter of the wire, in order to make the angle between the filaments and the axis of the wire approximately the same in all cases—of the order of 45°. Reduction of this angle would enable a heavier bundle to be employed, and an increased rate of production to be obtained, but is undesirable as resulting in a layer of insulation that is liable to slip along the length of the wire and leave gaps in the insulation. By the use of the present invention, however, this disadvantage may be overcome, since, after coalescence, the filaments employed are bonded together and, to some extent, to the wire itself, and have little or no tendency to slip. In consequence the invention enables lapping yarns of larger deniers to be employed and to be disposed at a smaller angle to the axis of the wire, so that the rate of production may be correspondingly increased. For the purposes of the present invention, as in silk lapping, a single layer of filaments may be laid on the wire in the lapping operation, or two or even more layers, according to the gauge of the wire and the total thickness of insulation permissible.

After lapping the wire the filaments wound on the surface thereof are caused to coalesce. This is preferably effected by the application of heat, which may be employed either alone or with the assistance of a medium or high-boiling solvent or plasticiser to reduce the temperature necessary to bring about coalescence. If heat is employed alone to effect coalescence, the degree of coalescence effected may be sufficient to bring about an appreciable fusion of the filaments so that they form a transparent or semi-transparent covering of uniform thickness through which the wire can be seen. If coalescence is effected with the aid of a medium- or high-boiling solvent or plasticiser, a lower degree of coalescence may be effected, which allows the filamentary structure to remain in some degree, and gives a covering which is opaque or of dull lustre.

The application of heat to the wire after lapping may be effected in an enamelling furnace of the kind used for enamelling fine wires for use as electrical conductors, the wires being supplied from a creel carrying a number of supply packages and, after passing through the furnace, returning to the creel to be rewound. Such a furnace may be used without substantial modification, unless it is desired, on account of the nature of the insulating material employed and its behaviour at high temperature in the presence of air, to provide for the heating to take place in an inert gas. In such circumstances, appropriate provision may be made for the supply of inert gas to the furnace, and for preventing the gas from escaping unduly rapidly through the openings by which the wires enter and leave the furnace. Where cellulose acetate filaments are employed, a temperature of from 250° C.-320° C. is appropriate and a time of 1-25 seconds, according to the temperature employed and the degree of coalescence required. Thus, by running a wire of 28 standard wire gauge, covered with a double lapping of a 100 denier bundle of cellulose acetate filaments, at 9 ft. a minute through a furnace tube 40' in length at a temperature of 300° C. a well coalesced transparent lacquer-like covering is obtained, while with a temperature as low as 250° C. the filamentary structure is quite clearly visible. Again, good results may be obtained by exposing the lapped wire in a furnace at 290-300° C. for a period of 14 seconds, or at 305° C. for a period as short as 4½ seconds. Instead of a single run through the enamelling furnace, the lapped wire may be given two or more runs, at higher speeds so as to give a shorter exposure in each run than would be required in a single run.

Instead of using a standard type of enamelling furnace, other means may be employed for the purpose of applying heat to the lapped wire. Thus, the wire may be heated by radiant heat emitted by infra-red lamps, the radiation being suitably focussed on the line of travel of the wire being heated. For this purpose a reflector in the form of a cylinder of elliptical cross section may be employed, the filament of the infra-red lamp being at one focus of the elliptical section and the path of the wire being at the other.

In order to reduce the temperature necessary to effect coalescence, a high-boiling solvent or plasticiser may be employed. High-boiling plasticisers, such as dicesyl glyceryl ether or the acetate thereof, or diethyl phthalate, or triacetin, may be employed in quantities up to 5% of the weight of the yarn or even more, the plasticiser being applied by running the lapped wire through

a solution of the plasticiser, e. g. in methylated spirit, the methylated spirit being evaporated by passing the wire through warm air at about 100° C., thus leaving the plasticiser in the filaments. It is preferable, however, if a liquid agent is to be employed, that it should be a low-boiling plasticiser, such as diacetone alcohol or glycol monoacetate which, as described in connection with high-boiling plasticisers, may be applied in solution, for example in methylated spirit. Thus, a solution of 55 parts of diacetone alcohol in 45 parts of methylated spirit may be applied to the covered wire by running the wire through the liquid so as to give it a time of immersion of 10 seconds, after which the wire is passed through hot air at a temperature of 120-150° C. or more. In the course of heating the methylated spirit is readily evaporated, but the diacetone alcohol evaporates much more slowly, and has the effect, in conjunction with the temperature to which the wire is exposed, of coalescing the filaments thereon. As an alternative to applying the low-boiling plasticiser to the lapped wire, the wire itself may be run through the liquid to be applied immediately prior to lapping and continuously with that operation. Again, the application of heat may be effected continuously with the lapping operation, a suitable length of run and temperature being employed corresponding with rate of travel of the yarn as it is lapped.

While, as stated above, it is preferred to employ heat for coalescing the filaments, coalescence can be brought about by relying wholly on the action of a softening agent for the substance of the filaments, the agent being applied to the filaments by running the lapped wire through a bath of the agent. Where cellulose acetate filaments are employed, convenient softening agents for use alone are acetone or methyl ethyl ketone, though any other of the well-known softening agents or plasticisers for cellulose acetate may be employed, provided that a time of immersion is allowed appropriate to the softening power of the agent used. Diluents, such as benzene or alcohol, may be employed to modify the severity of the solvent employed, or, if desired, a solution in low concentration say 1/2-2%, of the substance of the filaments may be used. After having passed through the softening agent, the emerging wire may be dried by allowing a convenient length of run in air which may take place in a tube or chamber from which the air is removed for subsequent solvent recovery. The product then resulting is an electrical conductor having an insulating covering intermediate in form between a filamentary lapping and a layer of varnish or enamel, the filamentary nature and structure of the covering being to some extent retained while the adjacent turns of filament in the lapping are coalesced and caused to unite with one another to form a covering that is continuous along the length of the wire.

The filaments employed for the purposes of the present invention may be dyed or otherwise given a distinctive appearance, e. g. for the purpose of distinguishing from one another, wires intended for different purposes, or for identifying different wires assembled in the form of a cable. Care should be taken, however, that the methods and materials used for this purpose should not be such as to impair the insulating properties of the filaments, and that the distinctive effect, if required in the finished product, should not be destroyed by the step of coalescing the filaments,

5 e. g. by the application of heat. Dyes may be applied to the wires after they have been lapped with the filaments, in order to colour the filaments, and this may be done in some circumstances by incorporating a suitable dye in a solvent or softening agent that is to be used to effect or facilitate coalescence of the filaments. Thus, where a mixture of equal parts by volume of triacetin and methylated spirit is used as a solvent or softening agent, a red colour may be given to the filaments by adding to the liquid 1.25 grams per litre of alpha-ethanolamino-anthraquinone, or a blue colour by adding the same proportion of 1:4-di(methylamino)-anthraquinone, or a yellow colour by adding the same proportion of 4-acetylamino-2'-hydroxy-4' phenylazobenzene. Other colours may be obtained by using mixtures of the above dyes. Pigmented filaments, obtained by incorporating a finely divided pigment such as titanium dioxide in the spinning solution from which the filaments are formed, may be used for the purpose of the present invention, and may be especially convenient when a thorough coalescence by means of heat alone is effected, whereby unpigmented filaments would form a transparent coating and the insulated wire might be mistaken at sight for bare wire.

10 The method of insulating according to the invention may be employed by itself, especially on very fine wires of from 47-50 gauge, or in other cases where very thin layers of insulation are required. The method may also, however, be employed in conjunction with other methods of insulating. For example, where normally a double lapping of silk might be employed, as on wires of the order of from 30 to 46 gauge, the inner layer of silk may be replaced by a lapping of filamentary materials coalesced in accordance 15 with the present invention and an outer lapping of silk may be superimposed on the inner layer so provided. Again, an insulating covering may be superposed, by the method according to the invention, on a coating of enamel previously applied.

20 By means of the invention, electrical conductors, and especially fine wires of the order of 30-35 gauge, can be insulated very satisfactorily. Among the advantages that may be obtained in conductors insulated in accordance with the invention are the previously mentioned advantage of avoiding slipping of a filamentary layer of insulating material along the length of the wire 25 so as to leave bare places, and the relatively low cost, as compared with silk, of the filamentary materials that are employed. At the same time, materials may be selected that give insulating layers of which the desirable electrical qualities, particularly the insulation resistance and breakdown value in voltage per unit thickness, are equal, and even superior to those of silk coverings. Advantage may be taken of this fact, and also of the fact that filaments as fine as, and even finer than, silk may be used, to obtain a product in 30 which the coverings are thinner than silk coverings having the same resistance and breakdown values. Uniformity of thickness, a property of particular importance where thin coverings are concerned, is another advantage that may be obtained by means of the invention, especially when heat is employed as the softening agency and more especially when heat is employed alone. The insulating material being initially distributed in a solid state uniformly round the wire, and the subsequently induced fluidity necessary to bring

about coalescence being only slight in degree and not long maintained, the material has neither a great tendency nor a sufficient time to flow under gravity towards one side of the wire, as is apt to occur when wires are insulated by enamelling. The initial uniformity of the coating may consequently be retained during coalescence and in the final product. Another important property that may be imparted to the insulating covering by means of the invention is resistance to mechanical abrasion. In this respect again, the advantage is best obtainable by the use of heat, and preferably heat only, as the softening agency, the degree of abrasion resistance depending upon the temperature and time of exposure with which coalescence is effected. The following is an example of the manner in which the invention may be carried out:

*Example.*

Copper wire of 36 S. W. G. (.0076 inch diameter) lapped with a single covering of cellulose acetate yarn of 50 denier containing 50 filaments, was passed once at a speed of 54 feet per minute through a furnace tube 4 feet long, heated to 305° C.

Some of the advantages mentioned above are illustrated by the following comparison

A covered wire A prepared as described in the example was compared by standard methods with a 36 S. W. G. wire B having a double covering of silk. The abrasion resistance was compared in two ways, by rubbing the wires in one case (a) with a polished round rod of  $\frac{1}{8}$ " diameter, and in the other (b) with a knife edge of 0.015" radius; the wire in each case being tensioned with a load of 100 grams. The following results were obtained:

|                                           | Wire A | Wire B |
|-------------------------------------------|--------|--------|
| Thickness of covering in mils.....        | 0.6    | 2.7    |
| Insulation resistance in kilomegohms..... | 75     | 75     |
| Breakdown volts.....                      | 425    | 450    |
| Breakdown value in volts per mil.....     | 708    | 168    |
| Abrasion resistance, number of rubs.....  |        |        |
| (a) 1,200                                 | 900    |        |
| (b) 554                                   | 646    |        |

It will be seen that, notwithstanding the comparative thinness of the covering of the wire A insulated in accordance with the present invention, its insulation resistance is the same as the

wire B and the breakdown voltage scarcely less, the breakdown value in volts per mil. being much greater. Again, the abrasion resistance as measured by a moderately severe abrasive action is actually greater for the wire A than for the wire B, and as measured by a more severe abrasive action is still of the same order in spite of the smaller thickness of material.

Having described our invention what we desire to secure by Letters Patent is:

1. Method of insulating wire for use as an electrical conductor, said method comprising lapping the wire with fine artificial filaments having a denier not greater than 1.5 and consisting of a thermoplastic material having electrically insulating properties, applying to the lapped wire a liquid softening agent for the substance of the filaments, and then subjecting the wire to the action of heat so as to cause the filaments on the wire to coalesce and form a continuous insulating cover for the wire.

2. Method of insulating wire for use as an electrical conductor, said method comprising lapping the wire with fine artificial filaments having a denier not greater than 1.5 and consisting of a thermoplastic material having electrically insulating properties, applying to the lapped wire a liquid containing a high boiling solvent or plasticiser for the substance of the filaments, and then subjecting the wire to the action of heat so

as to cause the filaments on the wire to coalesce and form a continuous insulating cover for the wire.

3. Method of insulating wire for use as an electrical conductor, said method comprising lapping the wire with fine artificial filaments having a denier not greater than 1.5 and consisting of a thermoplastic material having electrically insulating properties, applying to the lapped wire a liquid softening agent for the substance of the filaments, subjecting the wire to the action of heat so as to cause the filaments on the wire to coalesce and form a continuous insulating cover for the wire, and then lapping the insulated wire with an additional coating of non-thermoplastic filamentary material.

DONALD FINLAYSON.

ERNEST LESLIE GREENWOOD.

WILLIAM JOHN SIMPSON.